

1

2,762,509

**FLOTATION OF POTASH-CONTAINING SALTS  
USING BIVALENT, ALIPHATIC ALCOHOLS**

Rudolf Bachmann, Hannover, Germany, assignor to Kali-  
vertriebsstelle G. m. b. H., Hannover, Germany (Abt.  
Kaliorschungsstelle), a corporation of Germany

No Drawing. Application June 12, 1952,  
Serial No. 293,210

Claims priority, application Germany June 26, 1951  
8 Claims. (Cl. 209—166)

This invention relates to improvements in the flotation of potash-containing salts.

The method of recovering sylvite from crude potash salts by flotation is known. According to the conventional process, the flotation is effected with the use of normal primary amines having more than six carbon atoms as the gathering frother, i. e., the collector. These primary amines generally produce satisfactory results as far as the KCl yield and the amount of concentrate is concerned. The consumption of the flotation agents is, however, relatively large, and in many cases so large that the economy of the process is jeopardized, due to the high cost of the amines.

Such a method is described in U. S. Patent No. 2,088,325. In accordance with the method of this patent, for example, about 500 grams of an amine hydrochloride having 12 carbon atoms are required for each ton of the crude salt in the flotation of a sylvinitite. It should also be borne in mind that, as the number of carbon atoms of the amines increases, the consumption also increases.

There are basically two reasons for this high amine consumption, which is a multiple of the theoretical consumption.

First, the natural, crude potash salts frequently contain amounts of clay or other slime-forming secondary constituents in addition to the salt components. The secondary constituents absorb a large part of the collector which is intended for the flotation of the salt, and thus prevents its use for this purpose.

Secondly, a part of the amine added is consumed in the formation of the froth.

Attempts were made to overcome these disadvantages by partially removing these secondary constituents before the flotation itself. Such methods are described in U. S. Patents No. 2,288,497 and No. 2,364,520, in which a portion of the clay substances is removed before the crude salt is ground to a fine state. This, however, requires very cumbersome apparatus and a certain K<sub>2</sub>O loss is inherent in the process itself. Despite this partial removal of the secondary constituents, i. e., the slime, suitable measures must be taken in the flotation process itself to depress the remaining slime. In accordance with U. S. Patent No. 2,288,497, this depression of the remaining slime is effected by the addition of starch. In accordance with U. S. Patent No. 2,364,520, the depression is effected by the addition of methyl cellulose, cellulose xanthate, or cellulose acetate. About 300 to 450 grams of starch and about 400 to 800 grams of cellulose derivates are required for each ton of crude salt. These amounts, as can be seen, are extremely high and add considerably to the cost of the process, thus endangering its economic feasibility.

2

Other attempts to reduce the cost of the process included the use of pine oil for the production of the froth to reduce the amine consumption. These attempts, however, never met with any decisive success.

5 One object of this invention is the flotation of potash-containing salts with a reduced consumption of both the flotation amine and of the slime depresser. This, and still further objects, will become apparent from the following description:

10 It has now been very surprisingly found that the consumption of both the amine and the slime depresser can be very considerably reduced by adding an agent, which is synchronized with the depresser. Put in another way, it may be stated that when using like quantities of amine, 15 it is now very surprisingly possible to obtain greatly increased yields of the desired salts. It has been found, that the frothers, which are known as effective in flotation, also give good results in combination with amines and appropriate slime depressers, but we have found, 20 that only quite definitely polar-unpolar agents have this substantial improving action.

It was surprisingly found, that the bivalent aliphatic alcohols, having more than 5 carbon atoms, have proven particularly advantageous for this purpose.

25 The bivalent aliphatic alcohols used in the process of this invention include the alcohols from the hexylglycol up to the pentadecylglycol. The octylglycol has been found particularly successful. The addition of the bivalent aliphatic alcohols may be varied from 1 gram up 30 to 100 grams per ton crude salt. The best results are obtained by an addition of about 25 grams of a bivalent aliphatic alcohol per ton crude salt.

The bivalent aliphatic alcohols may be added at one or more points of the flotation apparatus, but it is preferred to feed the greater part into the first preflrothing cell.

The amounts of the other additional agents such as the amines and the frothers are the same as in known processes of flotation of potash containing salts.

40 The complete theoretical reasons for this new startling action have not yet been determined. The method of the improved results will, however, be illustrated by the following examples, which are given solely for this purpose and not limitation.

45

## EXAMPLE I

A slime-containing hartsalz was ground to a maximum grain size of 0.4 mm. and floated in its mother liquid 50 without prior slime-removal with the hydrochloride of a normal, primary amine, which consisted essentially of octadecyl amine. 100 grams of this material were added per ton of the crude salt. The froth concentrate was not refloated. The flotation results as obtained are shown 55 in Table 1 below.

Table 1

[Addition: 100 grams per ton of amine]

|                  | Weight Yield, percent | KCl Content, percent | KCl Quantity, g. | KCl Yield, percent |
|------------------|-----------------------|----------------------|------------------|--------------------|
| Concentrate..... | 18.1                  | 71.3                 | 12.9             | 64.1               |
| Tailings.....    | 81.9                  | 8.8                  | 7.2              | 35.9               |
|                  | 100.0                 |                      | 20.1             | 100.0              |

**3**  
**EXAMPLE II**

Example I was repeated, using 150 grams of the primary amine for each ton of the crude salt. The froth concentrate was not refloated. The flotation results are indicated on Table 2 below.

*Table 2*  
[Addition: 150 grams per ton of amine]

|                  | Weight Yield, percent | KCl Content, percent | KCl Quantity, g. | KCl Yield, percent | 10 |
|------------------|-----------------------|----------------------|------------------|--------------------|----|
| Concentrate----- | 24.3                  | 71.2                 | 17.3             | 81.5               |    |
| Tailings-----    | 75.1                  | 5.2                  | 3.9              | 18.5               |    |
|                  | 100.0                 |                      | 21.2             | 100.0              | 15 |

In both cases, the concentrates had the same KCl content. Upon, however, increasing the amount of amine to 150 grams per ton, the KCl yield rose from 64.1% to 81.5%. A further increase of the yield could only be obtained with very large additional amounts of amine.

**EXAMPLE III**

The same hartsalz was used as in Example I. The salt was prepared in the identical manner. 100 grams per ton of the identical amine were used for the flotation. In addition, 25 grams per ton of cellulose glycolate and 25 grams per ton of octylglycol were added. A substantial increase in the KCl content of the concentrate from 71.3 to 82.6 KCl was obtained. The KCl yield increased from 64.1% in Example I to 89.9%. These results are indicated in Table 3 below.

*Table 3*

[Addition: 100 grams per ton of amine, 25 grams per ton of cellulose glycolate, 25 grams per ton of octylglycol]

|                  | Weight Yield, percent | KCl Content, percent | KCl Quantity, g. | KCl Yield, percent | 10 |
|------------------|-----------------------|----------------------|------------------|--------------------|----|
| Concentrate----- | 22.5                  | 82.6                 | 18.6             | 89.9               |    |
| Tailings-----    | 77.5                  | 2.7                  | 2.1              | 10.1               |    |
|                  | 100.0                 |                      | 20.7             | 100.1              | 15 |

**EXAMPLE IV**

The same hartsalz was used as in Example I. The salt was prepared in the identical manner. 100 grams per ton of the identical amine were used for the flotation. In addition 25 grams per ton of cellulose glycolate and 25 grams per ton of hexylglycol were added.

A substantial increase in the KCl content of the concentrate up to 80.5% was obtained. The KCl yield increased from 64.1% in Example I to 88.4%. The results are indicated in Table 4 below.

*Table 4*

[Addition: 100 grams per ton of amine, 25 grams per ton of cellulose glycolate, 25 grams per ton of hexylglycol]

|                  | Weight Yield, percent | KCl Content, percent | KCl Quantity, g. | KCl Yield, percent | 10 |
|------------------|-----------------------|----------------------|------------------|--------------------|----|
| Concentrate----- | 22.5                  | 80.1                 | 18.1             | 88.4               |    |
| Tailings-----    | 77.5                  | 3.1                  | 2.4              | 11.6               |    |
|                  | 100.0                 |                      | 20.5             | 100.0              | 15 |

**EXAMPLE V**

The same hartsalz was used as in Example I. The salt was prepared in the identical manner. 100 grams per ton of the identical amine were used for the flotation. In addition 25 grams per ton of cellulose glycolate and 25 grams per ton of tetradecylglycol were added. A great increase in the KCl content of the concentrate up to 79.4% was obtained. The KCl yield increased from

**4**  
64.1% in the Example I to 87.6%. These results are indicated in the Table 5 below.

*Table 5*  
[Addition: 100 grams per ton of amine, 25 grams per ton of cellulose glycolate, 25 grams per ton of tetradecylglycol]

|                  | Weight Yield, percent | KCl Content, percent | KCl Quantity, g. | KCl Yield, percent |
|------------------|-----------------------|----------------------|------------------|--------------------|
| Concentrate----- | 22.8                  | 79.4                 | 18.1             | 87.6               |
| Tailings-----    | 77.2                  | 3.4                  | 2.6              | 12.4               |
|                  | 100.0                 |                      | 20.7             | 100.0              |

All the examples show that the addition of octylglycol in the flotation of potash containing salts results the optimal effects in regard as well with the KCl content of the concentrate as with the KCl yield.

It is thus seen that the slight addition of the bivalent, aliphatic alcohol in accordance with the invention, in addition to the depresser, very startlingly increases the flotation results obtained. With this particularly favorable combination of amines with cellulose glycolates and glycols, a desliming of the crude salt prior to the flotation is generally no longer necessary. In certain special cases this removal may have a favorable action on the process. In accordance with the invention, the purity of the concentrate and the yield are always substantially improved.

The process is applicable in the same manner to the flotation of sylvinites, carnallites and all crude salt mixtures, such as are frequently obtained in mining. It is also applicable to the intermediate and final products obtained in the so-called solution process, the same good results being obtained. The products containing greater amounts of sodium chloride which are obtained on vacuum cooling of hot solutions of sylvinite, hartsalz or carnallite are examples of intermediate products which may be used as starting materials for the process of this invention.

I claim:

1. In the method for the flotation of crude soluble salts in which a suspension of the ground salt in its mother liquid is floated by means of a normal primary amine salt collector with the addition of a depresser selected from the group consisting of cellulose derivative depressers and starch product depressers, the improvement which comprises simultaneously adding a bivalent, aliphatic alcohol ranging from hexylglycol to pentadecylglycol, and recovering a concentrate of a high salt content.

2. Improvement according to claim 1, in which said bivalent, aliphatic alcohol is octylglycol.

3. Improvement according to claim 1, in which said depresser is cellulose glycolate.

4. Improvement according to claim 1, in which said crude salt is selected from the group consisting of sylvinites, hartsalz, carnallites, and their mixed salts.

5. Improvement according to claim 1, in which said crude salts are the decomposition products of carnallite.

6. Improvement according to claim 1, in which said crude salts are selected from the group consisting of intermediate and final products of the solution process.

7. Improvement according to claim 1, in which the crude salts are floated with desliming before flotation process.

8. Improvement according to claim 1, in which the crude salts are floated without desliming before the flotation process.

70 **References Cited in the file of this patent**

**UNITED STATES PATENTS**

- |           |                 |               |
|-----------|-----------------|---------------|
| 2,251,217 | Woodhouse       | July 29, 1941 |
| 2,288,497 | Tartaron et al. | June 30, 1942 |
| 2,364,520 | Cole et al.     | Dec. 5, 1944  |